

1

3,817,753

DEVELOPMENT OF PHOTOGRAPHIC MATERIAL  
Jozef Frans Willems, Wilrijk-Antwerp, and Joseph Louis de Munck, Heide-Kalmthout, Belgium, assignors to Agfa-Gevaert, Mortsel, Belgium  
No Drawing. Continuation of abandoned application Ser. No. 573,797, Aug. 22, 1966. This application Sept. 30, 1971, Ser. No. 185,351  
Claims priority, application Great Britain, Oct. 7, 1965, 42,591/65

Int. Cl. G03c 1/06, 1/34, 5/30

U.S. Cl. 96—66.3

7 Claims

## ABSTRACT OF THE DISCLOSURE

Iodonium compounds having the formulae



wherein the aromatic nuclei can be substituted and X represents an anion utilized in a photographic silver halide emulsion, increase the rate of development of a developer combination comprising hydroquinone and polyoxyalkylene compounds, extend the development latitude in which screen prints of good quality can be produced within normal developing times, and do not fog the photographic silver halide emulsion.

This is a continuation of application Ser. No. 573,797, filed Aug. 22, 1966, now abandoned.

This invention relates to a development process and to combinations of substances influencing the development, used in this development process.

It is known that the development of continuous tone images by means of a hydroquinone-p-N-methyl-aminophenol developer is accelerated under the influence of polyoxyalkylene compounds having a molecular weight preferably above 1500. When, however, such polyoxyalkylene compounds are used in combination with a hydroquinone-formaldehyde bisulphite developer, as is known from the German Patent Application 1,141,531, filed Jan. 24, 1962 by Perutz Photowerke G.m.b.H., an increase of gradation together with a desensitisation is obtained. The latter combination is found to be very suitable for the development of light-sensitive materials for use in the graphic art on account of the very contrasty development obtained therewith.

It is also known that the development retardation caused when using the combination of polyoxyalkylene compounds with the above-mentioned type of developer can be neutralized and that the initial rate of development can be raised by using quaternary ammonium salts in conjunction with the above combination. However, quaternary ammonium salts especially in high concentrations have the disadvantage of fogging a light-sensitive silver halide material.

It has been found now that iodonium compounds and more particularly iodonium compounds according to the following structural formulae:



wherein

X- represents an anion e.g. a halogen anion, a nitrate anion, a bisulphate anion, or a benthotriazolium anion,

2

and wherein the aromatic nuclei of said compounds may be substituted e.g. with an alkyl radical, a halogen atom, an alkoxy radical, a cyano radical, an acyl radical, or an acylamino radical,

5 considerably increase the initial rate of development of a developer combination comprising hydroquinone and polyoxyalkylene compounds, extend the development latitude in which screen prints of good quality can be produced, within normal developing times, preferably not longer than 3 minutes, and do not fog the photographic silver halide emulsion.

These compounds influencing the development are preferably added to the composition of the light-sensitive silver halide emulsions in dissolved form in water or a mixture of water and water-miscible organic solvents, which do not impair the photographic characteristics of the emulsion.

However, these compounds can also be incorporated into the emulsion by imbibition by treating it with a solution containing these products or by diffusion from an adjacent water-permeable layer comprising these compounds.

The compounds influencing the development according to the present invention can be added to the light-sensitive silver halide emulsion during different preparation steps of the light-sensitive material. For example they can be incorporated therein by a separate addition or they can be added as a mixture with one or more ingredients used in the formation of the silver halide grains, during the physical or chemical ripening or during another step preceding the coating of the emulsion.

The compounds according to the above general formulae are preferably used in combination with water-soluble polyoxyalkylene compounds i.e. alkylene oxide condensation products as described e.g. in the U.S. Patent Specifications 1,970,578 by Conrad Schoeller and Max Wittwer, issued Aug. 21, 1934, 2,240,472 by Donald R. Swan, issued Apr. 29, 1941, 2,423,549 by Ralph K. Blake, William A. Stanton, Ferdinand Schulze, issued July 8, 1947, 2,441,389 by Ralph K. Blake, issued May 11, 1948, 2,531,832 by William A. Stanton, issued Nov. 28, 1950, 2,533,990 by Ralph K. Blake, issued Dec. 12, 1950, and the British Patent Specifications 920,637, filed May 7, 1959, 940,051, filed Nov. 1, 1961, 945,340, filed Oct. 23, 1961 by Gevaert Photo-Producten N.V., 991,608, filed June 14, 1961 by Kodak and the Belgian Patent Specification 648,710, filed June 2, 1964 by Gevaert Photo-Producten N.V. and the British Pat. No. 1,107,022, corresponding to U.S. Pat. No. 3,573,913.

50 The alkylene oxide condensation products together with the compounds influencing the development as described above can be added to the composition of the silver halide emulsion or to a water-permeable layer, which together with the emulsion layer forms part of a waterpermeable element.

The alkylene oxide condensation products and/or the compounds according to the above general formulae can also be added to the developing bath.

55 The compounds influencing the development are preferably added to the emulsion after the chemical ripening and just before the coating of the emulsion.

The optimum amount of alkylene oxide condensation product and iodonium compound according to the above formulae depends on the very compound, on the nature of the colloid binder of the silver halide grains and on the kind of silver halide in the emulsion. In general, however, the above alkylene oxide condensation products are added to the light-sensitive material in an amount of 100 mg. to 10 g. per mole of silver halide. When incorporated into the developer they are used in amounts ranging from 0.1 g. to 10 g. per litre of developer.

The amount of iodonium derivative incorporated into the light-sensitive material preferably ranges between 10 mg. and 20 g. per mole of silver halide. When added to the developing bath, the derivative is used preferably in an amount varying between 0.1 g. to 20 g. per litre.

The development acceleration and the increase of dot definition and of the development latitude obtained with the products according to the present invention can be combined with a chemical sensitisation by using in combination with the above-mentioned condensation products chemical sensitising agents such as sulphur-containing compounds, e.g. allyl isothiocyanate, allyl thiourea or sodium thiosulphate, reducing agents such as the tin compounds described in the Belgian Patent Specifications 493,-464, filed Jan. 24, 1950 and 568,687, filed June 18, 1958, by Gevaert Photo-Producten N.V., the imino-amino methane sulphonic acid compounds described in the British Patent Specification 789,823, filed Apr. 29, 1955 by Gevaert Photo-Producten N.V., or precious metal compounds such as gold, platinum, palladium, iridium, ruthenium and rhodium compounds. The sensitising action also manifests itself, of course, when combining the above-mentioned condensation products with the sensitising compounds present by nature in gelatin.

The compounds influencing the development according to the present invention can also be used in combination with stabilising agents for silver halide emulsions, such as mercury compounds and the compounds described in the Belgian Patent Specifications 571,916 and 571,917, filed Oct. 10, 1958 by Gevaert Photo-Producten N.V., and in combination with sensitising and stabilising cadmium salts in the light-sensitive material as well as in the developer.

Other water-soluble compounds, which also accelerate the development, such as those described, e.g. in the British Patent Specification 954,205, filed June 30, 1960 by Gevaert Photo-Producten N.V. can be applied together with the condensation products according to the present invention in a developing bath as well as in the light-sensitive material.

general formula can be used as fog-inhibiting compounds in the light sensitive material:



10 wherein:

each of  $\text{R}_1$  and  $\text{R}_2$  represents a hydrogen atom, an alkyl, an aralkyl, or an aryl radical, and  
 $\text{R}_3$  represents a hydrogen atom, an alkyl, a carboxy, or an alkoxy carbonyl group.

15 Such compounds can be prepared starting from 1 mole of  $\beta$ -ketoester or an  $\alpha$ -ethoxymethylene- $\beta$ -ketoester with 1 mole of a suitable 3-amino-1,2,4-triazole. By way of example of such derivatives 5-methyl-7-hydroxy-s-triazolo (1,5-a)-pyrimidine can be mentioned.

20 Other agents such as hardening agents, wetting agents, plasticisers, developing agents, and optical sensitising agents can be incorporated into the emulsion in the usual way.

25 The combination of products influencing the development according to the present invention can preferably be used in the development of silver chloride and silver bromochloride emulsions with a hydroquinone-formaldehyde-bisulphide developer, but it can also be used advantageously in the development of other emulsion types in 30 combination with other developers.

The following example illustrates the invention.

#### EXAMPLE

35 After ripening of a green-sensitised silver chlorobromide emulsion (35 mole percent of bromide) containing 5-methyl - 7 - hydroxy-s-triazolo-(1,5-a)-pyrimidine and cadmium chloride the compounds listed in the following Table 1 are added thereto. After the addition of the usual

TABLE 1

Development time (in min.)

| Mg. of ingredients per mole of silver halide      | 2½             |     | 3     |      | 3½  |       | 2½   |     | 3     |      | 3½  |       |     |
|---------------------------------------------------|----------------|-----|-------|------|-----|-------|------|-----|-------|------|-----|-------|-----|
|                                                   | Dot definition | Fog | Speed | γ    | Fog | Speed | γ    | Fog | Speed | γ    | Fog | Speed | γ   |
| 1 100 mg. of compound 1                           | 1.8            | 2   | 3     | 0.01 | 84  | 13    | 0.01 | 90  | 7.9   | 0.01 | 100 | 84    | 8.3 |
| 2 100 mg. of compound 1 and 100 mg. of compound 2 | 2.5            | 1.5 | 1     | 0.01 | 35  | 12.5  | 0.01 | 58  | 12    | 0.01 | 87  | 12.3  |     |
| 1 100 mg. of compound 3                           | 1.8            | 2   | 3     | 0.01 | 84  | 12.7  | 0.01 | 100 | 9.1   | 0.01 | 100 | 8.1   |     |
| 2 100 mg. of compound 3 and 100 mg. of compound 2 | 2.5            | 1.5 | 1     | 0.01 | 18  | 8.3   | 0.01 | 38  | 8.7   | 0.01 | 76  | 14    |     |
| 1 110 mg. of compound 4                           | 1.6            | 1   | 1     | 0.01 | 29  | 8.2   | 0.01 | 50  | 11.3  | 0.01 | 84  | 25    |     |
| 2 110 mg. of compound 4 and 240 mg. of compound 5 | 1.8            | 2   | 3     | 0.01 | 84  | 12.5  | 0.01 | 100 | 9.5   | 0.01 | 100 | 8.4   |     |
| 3 110 mg. of compound 4 and 240 mg. of compound 5 | 2.5            | 1.5 | 1     | 0.01 | 35  | 10    | 0.01 | 58  | 13.2  | 0.01 | 87  | 13.5  |     |
| 1 110 mg. of compound 4                           | 1.6            | 1   | 1     | 0.01 | 66  | 11.7  | 0.01 | 84  | 15.5  | 0.01 | 87  | 10.9  |     |
| 2 110 mg. of compound 4 and 190 mg. of compound 2 | 4              | 2   | 2     | 0.01 | 22  | 6.3   | 0.01 | 66  | 12.2  | 0.01 | 100 | 9.7   |     |
| 3 160 mg. of compound 4 and 190 mg. of compound 2 | 4              | 4   | 1.5   | 0.01 | 18  | 10.6  | 0.01 | 54  | 11.3  | 0.01 | 81  | 12.4  |     |
| 4 180 mg. of compound 6                           | 4              | 2   | 1.5   | 0.01 | 32  | 10.8  | 0.01 | 34  | 8     | 0.01 | 71  | 10.3  |     |
| 5 160 mg. of compound 6 and 195 mg. of compound 2 | 4              | 1   | 1     | 0.01 | 62  | 11.8  | 0.01 | 84  | 11    |      |     |       |     |

Together with the above-mentioned condensation products, derivatives of tetra-azaindenes having the following 75 wetting agent, of 25% by weight of polyethyl acrylate as plasticiser calculated on the weight of gelatin, and of

hardening agent such as formaldehyde and glyoxal the emulsion samples are coated in the same way on a cellulose triacetate support and dried. The latex-plasticiser consists in a latex of 20% by weight of poly(ethyl acrylate) prepared according to known techniques by emulsion polymerisation in the presence of 3% by weight calculated on the monomer of the sodium salt of poly(ethylene-oxyoctylphenol) sulphonic acid wherein three ethylene-oxy units are present, 1% by weight of the sodium salt of the sulphuric acid ester of dodecyl alcohol and 2% of the condensation product of oleic acid and methyl taurine.

All of the samples are exposed in the same way through a grey wedge and a glass screen to a light source with a colour temperature of 3700° K. and developed at 19° C. in a bath comprising:

|                              |     |
|------------------------------|-----|
| Sodium bisulphite            | 1.5 |
| Hydroquinone                 | 17  |
| Formaldehyde bisulphite      | 60  |
| Anhydrous sodium carbonate   | 60  |
| Anhydrous sodium bicarbonate | 15  |
| Potassium bromide            | 1   |
| Water to 1000 ml.            |     |

The dot definition is judged visually by comparison to standard materials, which in decreasing value of dot definition quality are defined with the numbers 1, 2, 3 and 4.

For judging the speed the light-sensitive materials are exposed through a grey wedge (with constant 0.01).

The speed, measured at a density 3 above fog, is on a percentage basis as compared with the speed attained after a development time of 3.5 minutes using an emulsion containing no development-influencing compound.

*Compound 1:* is a polycondensation product of 1 mole of maleic anhydride and 1 mole of polyethylene glycol having an average molecular weight of 2000 prepared in an analogous way to preparation 3 of the British Patent Specification 920,637 filed May 7, 1959 by Gevaert Photo-Producten N.V.

*Compound 2:* is a compound used according to the present invention having the following structural formula:



*Compound 3:* is a polyoxyethylene polymer according to the following structural formula:



wherein  $x$  is approximately 135.

*Compound 4:* is a polyoxyethylene polymer prepared according to preparation 7 of the U.K. Pat. No. 1,107,022, corresponding to U.S. Pat. No. 3,573,913.

*Compound 5:* is a compound used according to the present invention having the following structural formula:



*Compound 6:* is a polyoxyethylene polymer prepared according to preparation 3 of the U.K. Pat. No. 1,107,022, corresponding to U.S. Pat. No. 3,573,913.

United Kingdom Pat. No. 1,107,022 is assigned to Gevaert Photo-Producten, N.V., and describes the preparation of various polymeric materials, particularly polyoxyethylene polymers useful in photographic emulsions.

We claim:

1. Process for developing a photographic element containing a light-sensitive silver halide layer, said layer comprising a member of the group consisting of a silver chloride and a silver bromochloride emulsion, said process comprising exposing said photographic element, and developing said photographic element with an alkaline solution, a polyoxyalkylene polymer and an iodonium com-

ound corresponding to one of the following structural formulae:



wherein:

$\text{X}^-$  is an anion selected from the group consisting of halogen, nitrate, bisulfate, and benzotriazoline, and  $\text{Ar}$  is a phenyl radical.

2. Process according to claim 1, wherein the development is carried out with a hydroquinone-formaldehyde-bisulphite developer.

3. Process according to claim 1, wherein the iodonium derivative is present in the light-sensitive material in a range of 10 mg. to 20 g. per mole of silver halide.

4. Process according to claim 2, wherein the polyoxyalkylene polymer is present in the light-sensitive material in an amount ranging from 100 mg. to 10 g. per mole of silver halide.

5. Process according to claim 1, wherein the iodonium derivative is present in a developing bath in an amount varying from 0.1 to 20 g. per litre of developer solution.

6. A photographic light-sensitive silver halide element comprising a member of the group consisting of a silver chloride and a silver bromochloride emulsion, and containing an iodonium compound and a polyoxyalkylene polymer, said iodonium compound corresponding to one of the following structural formulae:



wherein:

$\text{X}^-$  is an anion selected from the group consisting of halogen, nitrate, bisulfate, and benzotriazoline, and  $\text{Ar}$  is a phenyl radical.

7. A photographic light-sensitive silver halide material according to claim 5, containing in addition to a polyoxyalkylene polymer and an iodonium compound a fog-inhibiting compound of the following general formula:



wherein:

each of  $\text{R}'_1$  and  $\text{R}'_2$  represents a hydrogen atom, an alkyl, aralkyl or aryl radical, and

$\text{R}'_3$  represents a hydrogen atom, an alkyl, a carboxy, or an alkoxy carbonyl group.

#### References Cited

##### UNITED STATES PATENTS

|           |         |           |        |
|-----------|---------|-----------|--------|
| 2,105,274 | 1/1938  | Steigmann | 96—95  |
| 2,848,330 | 8/1958  | Chechak   | 96—107 |
| 3,294,540 | 12/1966 | Goffe     | 96—107 |
| 3,518,085 | 6/1970  | Milton    | 96—107 |

#### OTHER REFERENCES

C. Abstr.: vol. 53, 16775c-d.

70 RONALD H. SMITH, Primary Examiner

M. F. KELLEY, Assistant Examiner

U.S. Cl. X.R.

UNITED STATES PATENT OFFICE  
CERTIFICATE OF CORRECTION

PATENT NO. : 3,817,753

DATED : June 18, 1974

INVENTOR(S) : Jozef Frans WILLEMS ET AL

It is certified that error appears in the above-identified patent and that said Letters Patent are hereby corrected as shown below:

Column 1, in the heading, in the inventors' names, "Jozef Frans Willems, Wilrijk-Antwerp" should read -- Jozef Frans Willems, Wilrijk-Antwerpen --;

Column 1, line 71, "bendotriazolium anion" should read -- benzotriazolium anion --.

Column 4, line 29, "bisulphide" should read -- bisulphite --.

Column 5, line 72, claim 1, "cholride" should read -- chloride --.

Column 6, line 43, claim 7, "claim 5" should read -- claim 6 --.

Signed and Sealed this

fourth Day of May 1976

[SEAL]

Attest:

RUTH C. MASON  
*Attesting Officer*

C. MARSHALL DANN  
*Commissioner of Patents and Trademarks*